

# United States Patent Office

2,940,855

Patented June 14, 1960

1

2,940,855

**SENSITIZATION OF PHOTOGRAPHIC EMULSIONS**  
Dorothy J. Beavers, Charles V. Wilson, and James L. Graham, Rochester, N.Y., assignors to Eastman Kodak Company, Rochester, N.Y., a corporation of New Jersey

No Drawing. Filed Nov. 27, 1957, Ser. No. 699,199

17 Claims. (Cl. 96—107)

This invention relates to the sensitization of photographic silver halide emulsions with certain quaternary ammonium salts, e.g., pyridinium and quinolium salts.

The sensitization of photographic emulsions with compounds containing quaternary nitrogen atoms has been known for many years as shown by the Carroll U.S. Patent 2,271,623, granted February 3, 1942. A representative quaternary salt sensitizing agent of that patent is the compound ethylene-bis-oxymethylpyridinium perchlorate.

We have discovered certain compounds containing quaternary nitrogen radicals which exhibit improved properties as sensitizing agents for silver halide emulsions. Emulsions containing the compounds of the invention are appreciably more stable than emulsions containing the mentioned quaternary compounds. Accordingly, upon the aging of emulsions containing the new sensitizing agents, less fog is developed and the emulsion speed is maintained. Also, photographic emulsions containing the new quaternary nitrogen compounds maintain their speed over a wider range of development conditions than do emulsions sensitized with previously known alkylene-bis-pyridinium salts such as decamethylene-1,10-bis-pyridinium perchlorate. Thus emulsions containing the latter compound as a sensitizing agent can be expected to lose an appreciable amount of speed when developed with a developing solution of high sulfite content of the order of 100 grams of anhydrous sodium sulfite per liter, whereas the emulsion speed is maintained in such developers when the emulsion is sensitized with the quaternary salts of the present invention.

When the emulsions are sensitized with the quaternary salts of the invention and are used in processes of color photography, that is, in multilayer color films adaptable to the reversal process of color photography, the first development step with the usual Metol-hydroquinone developer produces less fog than when the emulsions are sensitized with other quaternary salts such as that of the above Carroll invention.

It is interesting to note that Howe and Glassett British Patent 566,314 and Vanselow and James PSA Section B, 36—40 (1935), have shown that certain quaternary nitrogen salts such as n-dodecylpyridinium bromide, n-dodecyltriethyl ammonium bromide, etc. are not effective in increasing speed when development is carried out with a p-phenylenediamine as the developing agent such as used in color photography. In fact, it is shown by these workers that development with the p-phenylenediamine developing agent in the presence of the quaternary nitrogen salts retarded the development rate. The quaternary salts of the present invention when employed in the emulsions as sensitizing agents unexpectedly do not retard development rate when development is carried out with a p-phenylenediamine type developing agent.

The quaternary salt sensitizing agents of the invention are bis-quaternary salts having the following general formulas:

(I)  $\text{QROOCA}(\text{COOR}')_{n-1}\text{Q}'$

and

(II)  $\text{QRCOOA}(\text{OOCR}')_{n-1}\text{Q}'$

where Q and Q' represent the same or different organic radicals containing quaternary nitrogen atoms such as

2

trialkyl ammonium salt radicals and cyclammonium salt radicals, e.g., pyridinium salt radicals or quinolium salt radicals. R and R' represent the same or different radicals, which may be alkylene, such as  $-(\text{CH}_2)_n-$ , and including a carbon chain separated by other atoms such as O or S, e.g.,

$-(\text{CH}_2)_n\text{O}(\text{CH}_2)_n-$  or  $-(\text{CH}_2)_n-\text{S}-(\text{CH}_2)_n-$

n and n' being integers of from about 1 to 10. The total chain length of R and R' must be such that the number of "atoms" in the linear chain joining Q to Q' does not exceed about 30. (The term "atoms" as used herein refers solely to the actual elements that compose the chain and not to any groups that these elements may carry.

15 For example,  $-(\text{CH}_2)_{10}-$  is considered to be a 10-atom chain, the hydrogen atoms being disregarded;  $-(\text{CH}_2)_5\text{CONH}(\text{CH}_2)_5-$  is a 12-atom chain; the oxygen, and hydrogen atoms being disregarded). A compound of the above structure wherein the chain contains 34 atoms has been found not to be useful as a sensitizing agent. Likewise compounds having less than about 14 atoms in the chain are not very useful sensitizing agents the sensitizing activity of the compounds decreasing rapidly in compounds having less than about 14 or more than about 30 atoms in the linear chain connecting Q to Q'. In a preferred embodiment of the invention, therefore, the compounds contain from about 14 to about 30 atoms in the chain.

In Formulas I and II above, group A represents a linear 30 chain of one or more atoms of carbon which may or may not contain sulfur, oxygen or nitrogen as an intermediate linkage. Since n represents the positive integers 1 or 2, when n equals 1, Formulas I and II represent a group of compounds having the formulas

35 (III)  $\text{QROOCAQ}'$   
(IV)  $\text{QRCOOAQ}'$

When n equals 2, Formulas I and II above represent a 40 very important class of compounds having the general formulas

(V)  $\text{QROOCACOOR}'\text{Q}'$   
(VI)  $\text{QRCOOAOOCR}'\text{Q}'$

In the above formulas the number of atoms comprising A is obviously limited by the number of atoms in groups R and R' since as mentioned above, the total number of atoms in the linear chain connecting Q to Q' must not exceed about 30. Thus, in Formulas V and VI, A may contain as many as about 24 atoms in a linear chain when R and R' are methylene groups. Similarly in Formulas III and IV, A may contain about 27 atoms in a linear chain when R represents a methylene group. Chains of carbon, nitrogen, oxygen or sulfur atoms represented by A are as follows:



3 when  $n$  and  $n'$  are positive integers of the order of 1 to 10 selected so that the linear chain between Q and Q' contains from about 14 to about 30 atoms. The examples hereinafter provide compounds in which A has been varied as above to obtain very effective sensitizing agents.

Compound I:



Compound II:



Compound III:



Compound IV:



Compound V:



Compound VI:



Compound VII:



The compounds of the invention having the above 40 formulas may be prepared as follows:

Bis-ester (sym):



Bis-ester (unsym):



Inverse bis-ester (sym):



The unsymmetrical inverse bis-ester is prepared similarly by reacting separately with  $\text{XR}'\text{COOH}$  and  $\text{XR}'\text{COCl}$  or  $\text{XR}'\text{COOH}$ .

Monoesters:



The halide intermediates  $\text{XROOCAX}$  and  $\text{XRCOOAX}$  are prepared as follows:



5 Representative bis-quaternary salts of the invention may be prepared as described in detail below.

MONOESTER (COMPOUND V):

1-bromo-22-chloro-11-oxo-12-oxadocosane



10 Decamethylene chlorohydrin, 19.3 g. (0.10 mole), was dissolved in 200 ml. of dry benzene. The solution was chilled to 10° and 28.3 g. (0.10 mole) of  $\omega$ -bromo-undecanoyl chloride added slowly to the mixture, keeping the temperature at 10°. After stirring for two hours, the benzene solution was slurried with 100 ml. of water. 15 The benzene layer was concentrated on the Rinco evaporator to yield a yellow oil which solidified upon cooling. M.P. 30-32°. The ester may separate from the benzene solution when washing with water. The solid was dissolved in acetone, ether added to the cloud point, and the solution chilled. Beautiful white platelets (33.5 g., 76 percent), M.P. 34-36° were obtained.

Analysis.—Calc. for  $\text{C}_{21}\text{H}_{40}\text{BrClO}_2$ : C, 57.3; H, 9.1; Br, 18.2. Found: C, 58.0; H, 9.0; Br, 17.8.

25 12-oxa-11-oxadocosane-1,22-bis(pyridinium perchlorate)



30 Thirty ml. of pyridine and 10.0 g. (0.023 mole) of 1-bromo-22-chloro-11-oxo-12-oxadocosane were refluxed together for two hours. The excess pyridine was removed on the steam bath under vacuum, leaving a yellow oil. The oil was dissolved in 10 ml. ethanol and dry ether added to precipitate the product as a yellow oil. The solvent was decanted and the purification repeated.

The yellow oil was dissolved in 25 ml. of methanol, and a solution of 7.7 g. (0.055 mole) of sodium perchlorate monohydrate in 50 ml. of methanol was added, and the solution concentrated on the steam bath to about 25 ml. Acetone was added and the inorganic salt filtered off.

The filtrate was chilled in Dry-Ice-acetone while gradually diluting with dry ether. A white crystalline solid, M.P. 54-57° (cloudy), was filtered off. The solid was dissolved in acetone, filtered to remove any traces of inorganic salt, and the clear solution chilled while adding ether. After two recrystallizations, 9.7 g. (62 percent) of tiny white needles of M.P. 60-62.5° were collected. 55 The product gave a clear foaming solution in water. An analytically pure sample was obtained from acetone-ether.

Analysis.—Calc. for  $\text{C}_{31}\text{H}_{50}\text{N}_2\text{Cl}_2\text{O}_{10}$ : C, 54.6; H, 7.3; N, 4.1. Found: C, 54.1; H, 7.5; N, 4.0.

55 BIS-ESTER (SYM) (COMPOUND III):

7,18-dioxa-8,17-dioxotetraicosane-1,24-dichloride



60 Hexamethylene chlorohydrin (27.3 g., 0.20 mole) was dissolved in 50 ml. of dichloromethane in a 300-ml. flask equipped with stirrer and dropping funnel. Sebacyl chloride (24 g., 0.10 mole) was added slowly through the dropping funnel; the temperature rose to 40°. The solvent was allowed to distill off carrying with it the hydrogen chloride formed in the reaction. Additional solvent was added and allowed to escape along with the remaining hydrogen chloride. The pale yellow oil was dissolved in 100 ml. of ether and washed with water to remove any hydrogen chloride in the product. The ether layer was dried over sodium sulfate. Upon removal of the ether, a light yellow oil was obtained which crystallized upon chilling in an ice bath. The white solid, 41.2 g. (94 percent), melted at 12-15°.

70

7,18-dioxa-8,17-dioxotetracosane-1,24-bis(pyridinium perchlorate)



A mixture of 25 ml. of pyridine and 11.0 g. (0.025 mole) of the bis-ester above was refluxed for six hours. The excess pyridine was removed on the steam bath under vacuum. Methanol was added to the orange oil and this removed under vacuum to eliminate last traces of pyridine. The oily pyridinium chloride was then dissolved in 25 ml. of methanol, heated to boiling, and treated with a hot solution of 8.4 g. (0.06 mole, 20 percent excess) of sodium perchlorate monohydrate in 25 ml. of methanol. Immediately sodium chloride precipitated from the reaction and was filtered off. The mixture was concentrated to about 20 ml., cooled, and the remaining sodium chloride filtered off. The methanol solution was chilled in a Dry Ice-acetone bath with vigorous scratching while ether was slowly added. A white solid precipitated from solution. The solid was dissolved in acetone and crystallized by chilling in a Dry Ice-acetone mixture, 12.9 g. (72 percent; melting point 112-115°). An analytical sample of the bis-ester was obtained by repeating the crystallization. The melting point was unchanged.

*Analysis.*—Calc. for  $\text{C}_{32}\text{H}_{50}\text{N}_2\text{Cl}_2\text{O}_{12}$ : C, 53.0; H, 6.9; N, 3.9; Cl, 9.8. Found: C, 53.1; H, 7.1; N, 3.7; Cl, 10.8.

Compounds I and II are prepared similarly by use of the corresponding chlorohydrin and diacid halide.

COMPOUND IV

7,10,13,16,19-pentoxa-6,20-dioxopentacosane-1,25-dibromide

Ten grams (0.052 mole) of tetraethyleneglycol, 20.0 g. (0.103 mole) of  $\omega$ -bromocaproic acid, 0.1 g. of p-toluenesulfonic acid, and 200 ml. of dry p-xylene were added to a 500-ml. flask equipped with Dean-Stark trap and condenser. After 4 hours of vigorous refluxing, the theoretical amount of water had been collected in the trap. The yellow solution was washed twice with water and dried over  $\text{Na}_2\text{SO}_4$ . The solvent was removed under vacuum on the steam bath. The resulting orange water-insoluble oil (21.5 g., 76 percent) was used in the next step without purification.

COMPOUND V

7,10,13,16,19-pentoxa-6,20-dioxopentacosane-1,24-bis(pyridinium perchlorate)

In a 100-ml. flask, 20 g. (0.036 mole) of 7,10,13,16,19-pentoxa-6,20-dioxopentacosane-1,25-dibromide (above) and 50 ml. of pyridine were refluxed for 4 hours. The excess solvent was removed on the steam bath under vacuum. The dark orange oil was slurried several times with ether, and the ether decanted in order to remove traces of pyridine in the oil.

A small sample, 4.0 g. of the above pyridinium bromide, was dissolved in 20 ml. of methanol and added to a solution of 1.8 g. of sodium perchlorate monohydrate in 25 ml. of acetone. The solution was concentrated to a sticky yellow residue. Treatment with acetone dissolved the quaternary salt. The insoluble sodium bromide was removed by filtration. On removal of the acetone there was obtained 3.6 g. (86 percent) of a tan water-soluble oil.

*Analysis.*—Calc. for  $\text{C}_{30}\text{H}_{46}\text{Cl}_2\text{N}_2\text{O}_{15}$ : C, 48.3; H, 6.2; N, 3.8; Cl, 9.5. Found: C, 47.5; H, 6.8; N, 3.6; Cl, 10.1.

COMPOUND VI

7,18-dioxa-6,19-dioxotetracosane-1,24-dibromide

To a solution of 8.7 g. (0.05 mole) of 1,10-decanediol and 14 g. of triethylamine in 50 ml. of benzene and 250 ml. of dichloromethane was added 21.3 g. (0.10

mole) of  $\omega$ -bromocaproic chloride in 60 ml. of benzene. The addition was rapid enough to maintain gentle refluxing. The mixture was allowed to stand for 48 hours, during which time triethylamine hydrochloride had precipitated and it was filtered off. The product was concentrated to a yellow residue on the steam bath under vacuum.

Approximately 150 ml. of water were added to the syrup, and the ester extracted with three 200-ml. portions of ether. The ethereal extracts were dried over sodium sulfate. The bis ester (20 g., 76 percent) was obtained as a pale yellow oil, M.P. 2°.

*Analysis.*—Calc. for  $\text{C}_{22}\text{H}_{40}\text{Br}_2\text{O}_4$ : C, 50.0; H, 7.6; Br, 30.3. Found: C, 52.5; H, 7.8; Br, 26.6.

15 7,18-dioxa-6,19-dioxotetracosane-1,24-bis(pyridinium perchlorate)

A solution of 10 g. (0.019 mole) of 7,18-dioxa-6,19-dioxotetracosane-1,24-dibromide (above) and 25 ml. of dry pyridine was refluxed for 4 hours. The excess pyridine was removed on the steam bath under vacuum. The oil was slurried with ether several times, and the ether decanted to remove traces of pyridine. The oily salt was then dissolved in 30 ml. of methanol. This solution was added to a solution of 6.4 g. sodium perchlorate monohydrate in 50 ml. of acetone. The mixture was concentrated to about one-half the original volume and 50 ml. of acetone added. The sodium bromide precipitate was filtered off. The solution was chilled in Dry Ice-acetone with scratching and ether slowly added. The sticky, semisolid that formed was redissolved in 20 ml. of methanol and the above treatment repeated twice, giving 10 g. of white solid, M.P. 65-67.5°; softens 55° (73 percent).

An analytical sample was obtained from methanol-ethanol after two recrystallizations, M.P. 79.5-81.0°.

*Analysis.*—Calc. for  $\text{C}_{32}\text{H}_{50}\text{Cl}_2\text{N}_2\text{O}_{12}$ : C, 53.0; H, 6.9; N, 3.9; Cl, 9.8. Found: C, 54.5; H, 6.9; N, 4.6; Cl, 10.0.

COMPOUND VII

40 6,17-dioxa-7,16-dioxodocosane-1,22-bis(dimethylamine)

Ten milliliters of triethylamine and 5.2 g. (0.04 mole) of dimethylaminoamyl alcohol were dissolved in 100 ml. of dry ether. A solution of 4.8 g. (0.02 mole) of sebacyl chloride in 50 ml. of ether was slowly added. The resulting slurry was allowed to stand 48 hours. The precipitated triethylamine hydrochloride was filtered off and the solvent removed under vacuum. The oil was dissolved in ether, washed with water, and the ethereal solution dried over sodium sulfate. Concentration of the solution gave 6.8 g. (79 percent) of a yellow oil of M.P. -13 to -14°.

*Analysis.*—Calc. for  $\text{C}_{24}\text{H}_{48}\text{N}_2\text{O}_4$ : C, 67.2; H, 11.2; N, 6.5. Found: C, 63.9; H, 11.3; N, 6.3.

The analysis indicates that an amine hydrate may have formed.

55 6,17-dioxa-7,16-dioxodocosane-1,22-bis(trimethylammonium p-toluenesulfonate)

To a solution of 3.6 g. (0.0084 mole) of 6,17-dioxa-7,16-dioxodocosane-1,22-bis(dimethylamine) above, 3.5 g. (0.018 mole) of methyl p-toluenesulfonate in 25 ml. of ethanol was added. After the exotherm had subsided, the solution was refluxed for an hour on the steam bath. The solution was concentrated to about 15 ml. and ether slowly added with chilling in an ice bath. A sticky, white, hygroscopic solid formed. The solid was dissolved in 20 ml. of methanol, chilled, and ether slowly added with scratching. The white solid thus obtained was recrystallized again in the above manner to yield 3.0 g. (45 percent) of a hygroscopic solid of M.P. 144-145°.

A hygroscopic analytical sample of M.P. 143-145° was obtained from a methanol-ethanol solvent.

*Analysis.*—Calc. for  $\text{C}_{40}\text{H}_{68}\text{N}_2\text{O}_{10}\text{S}_2$ : C, 60.0; H, 8.5; N, 3.5; S, 8.0. Found: C, 56.9; H, 8.6; N, 4.1; S, 8.1.

The following example illustrates the use of the bis-

7  
quaternary salts of the invention in photographic emulsions:

EXAMPLE 1

A high-speed bromoiodide emulsion was prepared chemically sensitized with sulfur and gold compounds and optically sensitized with a cyanine dye. The amounts of the bis-quaternary nitrogen compounds shown in the table below were added to samples of the emulsion alone and together with an azaindene stabilizing agent. The emulsion samples were then coated, exposed on a sensitometer and developed for 5 minutes at 68° F. in the developer given below. The speed, gamma and fog values obtained by sensitometric evaluation of the developed samples are also shown in the table. The speed values shown are expressed as  $100(1 - \log E)$  where E is the exposure in meter candle seconds required to produce in the emulsion a density of 0.3 above fog.

|                          |       |      |
|--------------------------|-------|------|
| Water                    | cc    | 500  |
| Elon                     | grams | 2.5  |
| Sodium sulfite anhydrous | do    | 30.0 |
| Hydroquinone             | do    | 2.5  |
| Sodium metaperborate     | do    | 10.0 |
| Potassium bromide        | do    | 0.5  |

TABLE I

| Number | Feature                                                                           | Speed | γ    | Fog  |
|--------|-----------------------------------------------------------------------------------|-------|------|------|
| 4248   | Control                                                                           | 312   | 1.05 | 0.16 |
| 4253   | 5,12-Dioxa-6,11-dioxohexadecane-1,16-bis(pyridinium perchlorate) (I) 0.75 g./mol. | 331   | 1.26 | .17  |
| 4256   | 4-Hydroxy-6-methyl-1,3,3a,7-tetraazaindene (XXX) 3.0 g./mol.                      | 326   | 1.20 | .14  |
| 4265   | (XXX) 3.0 g./mol + (I) 0.75 g./mol.                                               | 338   | 1.33 | .17  |
| 4266   | (XXX) 3.0 g./mol + (I) 2.25 g./mol.                                               | 345   | 1.24 | .18  |

EXAMPLE 2

Emulsions were prepared and tested as in Example 1 except that the addenda shown in Table II were added.

TABLE II

| Number | Feature                                                                              | Speed | γ    | Fog  |
|--------|--------------------------------------------------------------------------------------|-------|------|------|
| 911    | Control                                                                              | 318   | 1.29 | 0.20 |
| 914    | 7,18-Dioxa-8,17-dioxotetracosane-1,24-bis(pyridinium perchlorate) (III) 0.75 g./mol. | 343   | 1.06 | .42  |
| 921    | 4-Hydroxy-6-methyl-1,3,3a,7-tetraazaindene (XXX) 3.0 g./mol.                         | 325   | 1.31 | .19  |
| 927    | (XXX) 3.0 g./mol + (III) 0.75 g./mol.                                                | 354   | 1.05 | .25  |
| 928    | (XXX) 3.0 g./mol + (III) 2.25 g./mol.                                                | 351   | 1.16 | .27  |
| 940    | (XXX) 3.0 g./mol + PEG 1,500 (XXXI) 0.75 g./mol.                                     | 342   | 1.19 | .20  |
| 943    | (XXX) 3.0 g./mol + (XXXI) 0.75 g./mol + (III) 0.75 g./mol.                           | 359   | 1.33 | .32  |

Sample 943 shows that additional speed increase may be obtained by addition of a polyethylene glycol of average molecular weight of 1500 (PEG 1500), or similar polyalkylene oxides having molecular weights greater than about 300.

EXAMPLE 3

Emulsions were prepared and tested as in Example 1 except that the addenda shown in Table III were added.

TABLE III

| Number | Feature                                                                                        | Speed | γ    | Fog  |
|--------|------------------------------------------------------------------------------------------------|-------|------|------|
| 5537   | Control                                                                                        | 314   | 1.08 | 0.17 |
| 5545   | 7,10,13,16,19-Pentoxa-6,20-dioxopentacosane-1,25-bis(pyridinium perchlorate) (IV) 0.75 g./mol. | 332   | 1.34 | .20  |
| 5546   | 4-Hydroxy-6-methyl-1,3,3a,7-tetraazaindene (XXX) 3.0 g./mol.                                   | 326   | 1.36 | .18  |
| 5560   | (XXX) 3.0 g./mol + (IV) 0.75 g./mol.                                                           | 339   | 1.32 | .20  |
| 5561   | (XXX) 3.0 g./mol + (IV) 2.25 g./mol.                                                           | 342   | 1.29 | .22  |

EXAMPLE 4

Emulsions were prepared and tested as in Example 1 except that the addenda shown in Table IV were added.

TABLE IV

| Number | Feature                                                                  | Speed | γ    | Fog  |
|--------|--------------------------------------------------------------------------|-------|------|------|
| 5      | Control                                                                  | 306   | 1.20 | 0.13 |
| 3938   | 12-Oxa-11-oxodocosane-1,22-bis-(pyridinium perchlorate) (V) 0.75 g./mol. | 293   | .81  | .55  |
| 3942   | 4-Hydroxy-6-methyl-1,3,3a,7-tetraazaindene (XXX) 3.0 g./mol.             | 318   | 1.39 | .13  |
| 3949   | (XXX) 3.0 g./mol + (V) 0.3 g./mol.                                       | 333   | .95  | .19  |
| 3950   | (XXX) 3.0 g./mol + (V) 0.75 g./mol.                                      | 327   | .91  | .20  |

EXAMPLE 5

The use of the bis-quaternary salts of the invention in color photography is illustrated in this example.

A sulfur and gold-sensitized gelatino-silver bromoiodide emulsion was ripened to maximum sensitivity. To this emulsion was added an optical sensitizing dye that extended the light sensitivity to 6000-7000 A. and a hydrophobic cyan color former suitably dispersed in a high boiling organic solvent. A portion of this liquid emulsion received no further treatment; to another portion was added one of the compounds described below. Both portions were coated on film support, and the dry films were exposed to red light in an intensity scale sensitometer. The exposed films were processed in the reversal color process 1 and the 5248 negative color process 2 with the results shown in the following table. The color process 2 was carried out as described by Hanson and Kisner JSMPT 61, 667-701 (1953), for the color negative film, type 5248, involving the steps of color development, fixation, silver bleaching and final fixation. Color process 1 was carried out at 75° F. as follows:

|    |                         |         |    |
|----|-------------------------|---------|----|
| 1. | Negative development    | minutes | 10 |
| 2. | Reversal flash exposure |         |    |
| 3. | Color development       | minutes | 15 |
| 4. | Silver bleaching        | do      | 8  |
| 5. | Fixing                  | do      | 3  |

40 The negative developer had the following composition:

|                                              |       |      |
|----------------------------------------------|-------|------|
| Water, 90° F. (32° C.)                       | liter | 1.0  |
| Sodium hexametaphosphate                     | grams | 2.0  |
| N-methyl p-aminophenol sulfate               | do    | 6.0  |
| Sodium sulfite, desiccated                   | do    | 50.0 |
| Hydroquinone                                 | do    | 6.0  |
| Sodium carbonate, monohydrate                | do    | 35.0 |
| Potassium bromide                            | do    | 2.0  |
| Sodium thiocyanate                           | do    | 1.5  |
| 0.5% solution (6-nitrobenzimidazole nitrate) | cc    | 12.0 |
| 0.1% solution of potassium iodide            | cc    | 10.0 |

The color developing solution above had the following composition:

|                                                                                       |       |       |
|---------------------------------------------------------------------------------------|-------|-------|
| 55 Water, 70 to 80° F. (21 to 27° C.)                                                 | liter | 1.0   |
| Benzyl alcohol                                                                        | cc    | 6.0   |
| Sodium hexametaphosphate                                                              | grams | 2.0   |
| Sodium sulfite, desiccated                                                            | do    | 5.0   |
| Trisodium phosphate                                                                   | do    | 40.0  |
| Potassium bromide                                                                     | do    | 0.25  |
| 0.1% solution of potassium iodide                                                     | cc    | 10.0  |
| Sodium hydrazide                                                                      | grams | 6.5   |
| (4-amino-N-ethyl-N-[β-methane-sulfonamidoethyl]m-toluidine sesquisulfate monohydrate) | grams | 11.33 |
| Ethylenediamine sulfate                                                               | do    | 7.8   |
| Citrazinic acid (2,6-dihydroxyisonicotinic acid)                                      | do    | 1.5   |

70 The silver bleaching solution above had the following composition:

|                        |       |      |
|------------------------|-------|------|
| Water 9° F. (32° C.)   | liter | 1.0  |
| Potassium dichromate   | do    | 5.2  |
| Potassium ferricyanide | do    | 70.0 |
| 75 Potassium bromide   | do    | 20.0 |

The fixing baths above had the following composition:

|                        |       |       |
|------------------------|-------|-------|
| Water, 80° F. (27° C.) | liter | 1.0   |
| Sodium thiosulfate     | do    | 150.0 |
| Sodium bisulfite       | do    | 20.0  |

TABLE V

| Number | Feature                    | Color Process 1 (Reversal) Speed Increase (A Log E) <sup>1</sup> | Color Process 2 (5248 Negative) Speed Increase (A Log E) <sup>2</sup> |
|--------|----------------------------|------------------------------------------------------------------|-----------------------------------------------------------------------|
| 19637  | Control                    |                                                                  |                                                                       |
| 19645  | Compound I 4.0 g./mol AgX  | +0.14                                                            | +0.18                                                                 |
| 19637  | Control                    |                                                                  |                                                                       |
| 19646  | Compound II 2.0 g./mol AgX | +0.08                                                            | +0.08                                                                 |

<sup>1</sup> Determined by measuring the shift of the reversal dye curve on the Log E axis at a given density below maximum density.

<sup>2</sup> Determined by measuring the shift of the negative dye curve on the Log E axis at a given density above minimum density.

## EXAMPLE 6

Emulsions were prepared and tested as in Example 1 except that the addenda shown in Table VI were added.

TABLE VI

| Number  | Feature                                                                                                     | Speed | $\gamma$ | Fog  |
|---------|-------------------------------------------------------------------------------------------------------------|-------|----------|------|
| 180,576 | Control                                                                                                     | 293   | 1.04     | 0.14 |
| 180,582 | 7,18-Dioxa-6,19-dioxotetracosane-1,24-bis(pyridinium perchlorate) (VI) .75 g./mol AgX.                      | 314   | 1.03     | 1.03 |
| 180,584 | 4-Hydroxy-6-methyl-1,3,3a,7-tetraazaindene (XXX) 3.0 g./mol AgX.                                            | 293   | 1.28     | .18  |
| 180,593 | (XXX) 3.0 g./mol+(VI) 0.15 g./mol                                                                           | 314   | 1.22     | .16  |
| 180,594 | (XXX) 3.0 g./mol+(VI) 0.75 g./mol                                                                           | 313   | .92      | .18  |
| 180,595 | (XXX) 3.0 g./mol+(VI) 3.0 g./mol                                                                            | 337   | .94      | .23  |
| 188,629 | Control                                                                                                     | 306   | 1.10     | .14  |
| 188,635 | 6,17-Dioxa-7,16-dioxodocosane-1,22-bis(trimethyl ammonium p-toluene sulfonate) (III) 0.75 g./mol AgX.       | 321   | 1.10     | .14  |
| 188,658 | 4-Hydroxy-6-methyl-1,3,3a,7-tetraazaindene (II) 3.0 g./mol AgX.                                             | 313   | 1.03     | .14  |
| 188,649 | (II) 3.0 g./mol+(III) 0.75 g./mol                                                                           | 317   | 1.15     | .15  |
| 188,650 | (II) 3.0 g./mol+(III) 3.0 g./mol                                                                            | 321   | 1.10     | .18  |
| 182,218 | Control                                                                                                     | 303   | 1.26     | .12  |
| 182,224 | 4,13-Dioxa-3,14-dithiophexadecane-1,16-bis(diethylmethylammonium p-toluene sulfonate) (IV) 0.15 g./mol AgX. | 311   | 1.28     | .18  |
| 182,239 | 4-Hydroxy-6-methyl-1,3,3a,7-tetraazaindene (II) 3.0 g./mol AgX.                                             | 305   | 1.06     | .10  |
| 182,251 | (II) 3.0 g./mol+(IV) 0.03 g./mol                                                                            | 310   | 1.24     | .12  |
| 182,250 | (II) 3.0 g./mol+(IV) 3.0 g./mol                                                                             | 313   | 1.14     | .22  |

The bis-quaternary salts described above can be used in emulsions in the manner of the examples in concentrations of the order of about 0.02 to 4 grams per mol of silver halide.

The emulsions may also be developed in the presence of the bis-quaternary salts by incorporating the salts into a developer solution. For example, when Compound I was incorporated into the negative developer (2 g. per liter) of color process 1 of Example 5 and a multilayer color film the emulsions of which contained coupler compounds was developed therein, speed increases were obtained particularly for the red-sensitive emulsion layer.

As indicated in the above examples, it may be desirable to incorporate a stabilizing agent into the emulsion sensitized with the bis-quaternary salts of the invention to reduce fog to normal levels. Azaindenes particularly suitable for this purpose are those described in the Carroll et al. U.S. patent applications Serial Nos. 627,135 and 627,136, filed December 10, 1956, for example, the following:

5-carboxy-4-hydroxy-1,3,3a,7-tetraazaindene,  
1,2-bis(4-hydroxy-6-methyl-1,3,3a,7-tetraazaindene-5-yl)ethane,  
1,2,3,4-tetrakis(4-hydroxy-6-methyl-1,3,3a,7-tetraazaindene-2-yl)butane,  
2-amino-5-carboxy-4-hydroxy-1,3,3a,7-tetraazaindene,  
4-hydroxy-6-methyl-1,3,3a,7-tetraazaindene,  
4-hydroxy-2-β-hydroxyethyl-6-methyl-1,3,3a,7-tetraazaindene,

5-carboxy-4-hydroxy-1,3,3a,7-tetraazaindene,  
7-hydroxy-1,2,3,4,6-pentazaindene,  
2,4-dihydroxy-6-methyl-1,3a,7-triazaindene,  
4-hydroxy-2γ-hydroxypropyl-6-methyl-1,3,3a,7-tetraazaindene and  
4-hydroxy-2-(4-pyridyl)-6-methyl-1,3,3a,7-tetraazaindene.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, The Theory of the Photographic Process, 1942, page 3). The sensitizing agents may be added at any stage, preferably after the final digestion.

The photographic emulsions which we use are of the developing-out type and best results have been obtained with gelatino-silver bromoiodide emulsions. However, emulsions of varying silver halide content may be used.

The emulsions are chemically sensitized by any of the accepted procedures in addition to sensitizing with the bis-quaternary salts of the invention. The emulsions may be digested with naturally active gelatin, or sulfur compounds may be added such as those described in Sheppard U.S. Patents 1,574,944 and 1,623,499, and Sheppard and Brigham U.S. Patent 2,410,689.

The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladite, which are used for sensitizing in amounts below that which produces any substantial fog inhibition, as described in Smith and Trivelli U.S. Patent 2,448,060, and as anti-foggants in higher amounts, as described in Trivelli and Smith U.S. Patents 2,566,245 and 2,566,263.

The emulsions may also be chemically sensitized with gold salts as described in Waller and Dodd U.S. Patent 2,399,083 or stabilized with gold salts as described in Damschroder U.S. Patent 2,597,856 and Yutzy and Leermakers U.S. Patent 2,597,915. Suitable compounds are potassium chloroaurate, potassium aurithiocyanate, potassium chloroaurate, auric trichloride and 2-aurosulfobenzothiazole methochloride.

The emulsions may also be chemically sensitized with reducing agents such as stannous salts (Carroll U.S. Patent 2,487,850), polyamines such as diethylene triamine (Lowe and Jones U.S. Patent 2,518,698), polyamines such as spermine (Lowe and Allen U.S. Patent 2,521,925), or bis-(β-aminoethyl) sulfide and its water-soluble salts (Lowe and Jones U.S. Patent 2,521,926).

The emulsions may also contain polyalkylene oxides and derivatives thereof such as the polyethylene glycols, in addition to the bis-quaternary compounds of the invention. Suitable polyalkylene oxides and polyalkylene oxide derivatives are described in Blake U.S. Patent 2,441,389, May 11, 1948, Blake et al. U.S. Patents 2,400,532, May 21, 1946, 2,423,549, July 8, 1947, and Jennings et al. U.S. Patent 2,577,127, December 4, 1951.

Other compounds useful for suppressing the fog level of the emulsion sensitized with the bis-quaternary compounds of the invention include the mercury compounds of Allen et al. U.S. Patent 2,728,663, Carroll and Murray U.S. Patent 2,728,664 and Leubner and Murray U.S. Patent 2,728,665, granted December 27, 1955, and the organic mercury compounds of Carroll et al. U.S. Patent 2,784,090, granted March 5, 1957.

Other stabilizing agents may be added to the emulsions containing the bis-quaternary salts such as the metal inorganic salts of U.S. patent application Serial No. 493,047, filed March 8, 1955, by J. E. Jones.

The chemical sensitizing agents and other addenda which we have described may be used in various kinds

of photographic emulsions, e.g., various silver salts may be used as the sensitive salt such as silver bromide, silver iodide, silver chloride or mixed silver halides such as silver chlorobromide or silver bromoiodide.

The dispersing agent for the silver halide may be 5 gelatin or other hydrophilic material such as collodion, albumin, cellulose derivatives or synthetic resins.

Since the coupler-containing emulsions sensitized as described with the bis-quaternary salts are adapted particularly for use in color photography, they will ordinarily comprise the emulsion layers of multilayer color films which emulsion layers are customarily differentially sensitized to the primary regions of the visible spectrum and contain coupler compounds producing dye images of colors complementary to the sensitivity of the emulsion layers. In a representative color film, one or more of the differentially sensitized emulsion layers may be sensitized with the bis-quaternary salts, and in a typical example, emulsions sensitized to the red, green and blue regions of the spectrum are superimposed on the support in that order and contain cyan, magenta and yellow color-forming coupler compounds respectively. A yellow filter layer such as yellow colloidal silver is advantageously interposed between the blue- and green-sensitive emulsion layers.

Since the emulsion layers sensitized with the bis-quaternary salts of the invention may contain coupler compounds they can be readily processed by well known methods to yield color negatives directly or positive images by means of well known reversal processes. That is, after initial exposure of the emulsion to a subject a developer of the p-phenylenediamine type will produce a colored image negative in respect to the subject. Likewise, if development of the emulsion layer is first carried out with a non-color-forming developer followed by reversal exposure of the residual silver halide and then color development, a colored positive is obtained as described in the examples above.

The coupler compounds used in the emulsion layers sensitized with the bis-quaternary salts, are any of the well known compounds which combine with the oxidation product of primary aromatic amino (p-phenylenediamines) silver halide color developing agents to form dyes, for example, the phenolic couplers of U.S. Patents 2,266,452, 2,362,598, 2,589,004, 2,474,293, 2,521,908, 2,423,730 and Fierke U.S. patent application Ser. No. 476,561; the pyrazolone couplers of U.S. Patents 1,969,479, 2,369,489, 2,600,788, 2,618,641, 2,511,231 and the open chain reactive methylene couplers of U.S. Patents 2,298,443, 2,652,329, 2,407,210, 2,271,238 and McCrossen et al. U.S. patent application Serial No. 575,099, filed March 30, 1956. Likewise, the emulsions may contain colored color-forming couplers as described in U.S. Patents 2,521,908, 2,706,684, 2,455,169, 2,694,703, 2,455,170 and 2,453,661.

The couplers may be dispersed in the emulsion layers of means of an oily coupler solvent according to the methods of U.S. Patents 2,304,940 and 2,322,027. However, if as may be the case, the couplers contain solubilizing groups such as  $\text{SO}_3\text{H}$  groups which render the couplers soluble in alkaline solution, the oily coupler solvent may be dispensed with and the couplers can be added to the emulsion from aqueous solutions as their alkali metal salts.

What we claim is:

1. A photographic silver halide emulsion containing a quaternary ammonium salt having a general formula of the class consisting of



and



wherein Q and Q' each represent radicals of the class consisting of



10 wherein  $\text{R}^2$ ,  $\text{R}^3$  and  $\text{R}^4$  represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals,  $n$  represents a positive integer of from 1 to 2, A represents a member of the class consisting of



25 and



30 wherein  $n'$  and  $n''$  represent positive integers of from about 1 to 10, there being from about 14 to about 30 atoms present in the shortest linear chain of atoms linking said quaternary nitrogen atoms.

2. A photographic silver halide emulsion containing a quaternary ammonium salt having the general formula



wherein Q and Q' each represent radicals of the class consisting of



45 and



50 wherein  $\text{R}^2$ ,  $\text{R}^3$  and  $\text{R}^4$  represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals, A represents an alkylene group of from 1 to 10 carbon atoms, there being from about 14 to about 30 atoms present in the shortest chain of atoms linking said nitrogen atoms.

60 3. A photographic silver halide emulsion containing a quaternary ammonium salt having the general formula



65 wherein Q and Q' each represent radicals of the class consisting of



70 and



wherein R<sup>1</sup>, R<sup>2</sup> and R<sup>3</sup> represent lower alkyl groups, Z represents the atoms necessary to complete a heterocyclic nucleus of the class consisting of pyridinium and quinolinium, R represents an alkylene group linked directly to the quaternary nitrogen atom of said radical, A represents an alkylene group of from 1 to 10 carbon atoms, there being from about 14 to 30 atoms present in the shortest linear chain of atoms linking the quaternary nitrogen atoms of said radicals.

4. A photographic silver halide emulsion containing a quaternary ammonium salt having the general formula



wherein Q and Q' each represent radicals of the class consisting of



and



wherein R<sup>2</sup>, R<sup>3</sup> and R<sup>4</sup> represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals, A represents an alkylene group of from 1 to 10 carbon atoms, there being from about 14 to about 30 atoms present in the shortest chain of atoms linking said nitrogen atoms.

5. A photographic silver halide emulsion containing the compound 5,12 - dioxa - 6,11 - dioxohexadecane - 1,16-bis(pyridinium perchlorate).

6. A photographic silver halide emulsion containing the compound 7,18 - dioxa - 8,17 - dioxotetracosane - 1,24-bis(pyridinium perchlorate).

7. A photographic silver halide emulsion containing the compound 7,10,13,16,19-pentaoxa-6,20-dioxopen-tacosane-1,25-bis(pyridinium perchlorate).

8. A photographic silver halide emulsion containing the compound 12 - oxa - 11 - oxodocosane - 1,22 - bis(pyridinium perchlorate).

9. A photographic silver halide emulsion containing the compound 7,18-dioxa-6,19-dioxotetracosane-1,24-bis(pyridinium perchlorate).

10. The emulsion of claim 1 further containing a coupler compound reactive with the oxidation products of a p-phenylenediamine silver halide developing agent to form a dye.

11. The emulsion of claim 2 further containing a coupler compound reactive with the oxidation products of a p-phenylenediamine silver halide developing agent to form a dye.

12. The emulsion of claim 3 further containing a coupler compound reactive with the oxidation products of a p-phenylenediamine silver halide developing agent to form a dye.

13. The emulsion of claim 4 further containing a coupler compound reactive with the oxidation products of a p-phenylenediamine silver halide developing agent to form a dye.

14. The emulsion of claim 2 further containing an azaindene stabilizing agent.

15. The emulsion of claim 3 further containing an azaindene stabilizing agent.

16. The emulsion of claim 4 further containing an azaindene stabilizing agent.

17. The emulsion of claim 1 wherein the silver halide is sulfur and gold sensitized.

#### References Cited in the file of this patent

#### UNITED STATES PATENTS

|    |           |                 |               |
|----|-----------|-----------------|---------------|
| 35 | 2,271,623 | Carroll         | Feb. 3, 1942  |
|    | 2,288,226 | Carroll et al.  | June 30, 1942 |
|    | 2,419,975 | Trivelli et al. | May 6, 1947   |
|    | 2,784,090 | Carroll         | Mar. 5, 1957  |

#### FOREIGN PATENTS

|    |         |           |               |
|----|---------|-----------|---------------|
| 40 | 115,971 | Australia | Oct. 15, 1942 |
|----|---------|-----------|---------------|